

M. A. ADAM, J. STEVENSON, A. T. MABBITT AND J. FIELDHOUSE,  
ELECTROLYSIS,  
APPLICATION FILED AUG. 31, 1920.

1,365,140.

Patented Jan. 11, 1921.



Fig.1



Fig.2



Inventors: *M. A. Adam*  
*J. Stevenson*  
*A. T. Mabbitt*  
*J. Fieldhouse*  
*H. R. Kerslake* ATTORNEY

# UNITED STATES PATENT OFFICE.

MATTHEW ATKINSON ADAM, JOHN STEVENSON, ALAN THOMAS MABBITT, AND JOHN FIELDHOUSE, OF LONDON, ENGLAND; SAID STEVENSON, SAID MABBITT, AND SAID FIELDHOUSE ASSIGNORS TO SAID ADAM.

## ELECTROLYSIS.

1,365,140.

Specification of Letters Patent. Patented Jan. 11, 1921.

Application filed August 31, 1920. Serial No. 407,222.

To all whom it may concern:

Be it known that we, MATTHEW ATKINSON ADAM, residing at 57 Lincoln's Inn Fields, London, W. C. 2, England, JOHN STEVENSON, residing at 28 Talbot road, Bayswater, London, W. 2, England, ALAN THOMAS MABBITT, residing at 3 Wallwood road, London, E. 11, England, and JOHN FIELDHOUSE, residing at 2 Byfield road, Walthamstow, London, E., England, all subjects of the King of Great Britain and Ireland, have invented certain new and useful Improvements Relating to Electrolysis, of which the following is a specification.

This invention relates to the electrolytic deposit of metals in non-coherent or loose crystalline form from solutions of metallic salts in a cell or cells having a rotating cathode.

The object of the invention is to provide improved constructions or combinations of apparatus for the above described purpose which enable improved practical results to be obtained.

The present invention, in brief, consists in the electrolytic deposition of metals in a non-coherent or loose crystalline form in a cell having a rotating cathode and employing a substantially uniform flow of electrolyte between the electrodes adapted to insure approximately uniform composition within the cell, and enable high current densities to be utilized.

Referring to the accompanying diagrammatic drawings,

Figure 1 represents a transverse sectional view of one form of construction of rotating cathode cell according to the present invention;

Fig. 2 is a similar view of a modification and

Fig. 3 is a similar view of a further modification.

In carrying this invention into effect in one form, by way of example, as indicated in Fig. 1, as applied to the electrolytic recovery of tin from iron chlorid solutions rich in tin and preferably rich in stannous chlorid as may be obtained by working the

process described in our co-pending application 407,250 corresponding to British ap-

plication No. 4838 of 1919, we construct the cell *c* with two carbon anode bars *a*, *b*, preferably of graphite which run the whole length of the cell. These are placed side by side, and hollowed out to form a trough of circular form concentric with the cathode drum *d*. At the lowest point they are bored through at *e* to form exits for the electrolyte. The bars are hollowed out to form the trough, and a number of communicating ways *f* of considerable width are formed adjacent to each upper edge or lip. These lips are grooved at *g* to receive a copper or like bar *h*, which serves to supply current to the anode bars. The copper bars are bored and countersunk at intervals to receive bolts *i* which pass down through the carbon bars *a*, *b*, and clamp them against a base board *j* suitably impregnated to prevent absorption of liquid. The communicating ways *f* are preferably formed beneath the edge in order to prevent the electrolyte passing through them from coming into contact with the bars *h*, and for a similar reason the bolts *i* are arranged to pass through the bars *a*, *b*, at solid sections between the communicating ways. Between the bars *a*, *b*, and the board *j*, is placed a rubber mat *l* for jointing purposes. The end cheeks of the cell are provided with supports for the drum, and are bolted against the ends of the carbon bars with similar rubber mats not shown. The longitudinal bolting may be effected by means of the copper bars *h*, in which case these project and are screwed to receive the clamping nuts not shown.

Outside of each of the carbon bars chambers *m*, *n* are formed to receive the electrolyte, and adjustable weirs *o* may be fitted along the edge of each carbon bar to regulate the flow of electrolyte, a uniform and evenly distributed flow being aimed at as far as possible.

The base board *j* is formed with a central duct *p* and a number of channels *q* leading to an outside chamber *r* which discharges over an outlet weir *s* of adjustable height.

The cathode drum *d* is placed in position, and is chosen of such a diameter as to leave

a segmental annulus  $t$  of suitable width for the electrolyte. It is also made longer than the anode bars, so as to extend beyond them at both ends. The electrolyte is supplied 5 through inlet orifices made say through the bottom of the cell, and flows over the inlet weirs  $o$  into the annular space  $t$  between the cathode and each of the anode bars. It then flows out through the bottom of the trough 10 at  $e$ , and into the outlet chamber  $r$ , where it passes over the outflow weir  $s$ .

The cathode drum is rotated at a suitable rate in relation to the rate of flow of the electrolyte, and to the current density employed (see, for example, our application 15 407,250 corresponding to British application No. 4838 of 1919).

A scraper plate  $v$  extends across the drum, and is supported preferably on a chute  $w$  20 which receives the tin as it is delivered by the scraper. The tin receiving chute  $w$  and scraper  $v$  are preferably mounted on hinges (not shown) so that they can be swung out of position when desired.

25 It is found that this cell works well with a cathode current density of about 2.5 amperes per square inch, the liquid flow and relative movement of cathode and electrolyte being adjusted as therein indicated for 30 the recovery of tin from a solution which has been employed to dissolve tin as described in our application 407,250.

This cell is applicable to the electro-deposition under considerable current densities 35 of all metals which under suitable conditions can be electro-deposited in loose or crystalline form.

According to a modified form of construction, as illustrated in Fig. 2, the trough 0 is formed by a graphite bar 20 hollowed out and provided with holes 21 along its base for exit of the electrolyte. The electrolyte passes into the trough cell from both sides over the edges of the graphite trough 20 from both sides 22 of the supply chamber and the exit passages 21 into a sump 23, whence it flows through a number of ways 24 to the outlet pipe 25.

The graphite bar is preferably impregnated with paraffin wax to exclude the electrolyte from the pores thereof. Electrical connection may be made conveniently by copper rods 2 passing through the end of the cell and entering the bar, care being 55 taken that no access to this connection is possible by the electrolyte. A convenient way of effecting good electrical connection is to drill a hole through the end wall of the cell penetrating partly into the anode, and 60 to ram into this hole finely powdered carbon impregnated with paraffin wax, finally making connection with this rammed powder externally to the cell.

The drum cathode 26 is mounted upon a

spindle above the trough 20, and thus may 65 be rotated during action of the cell with part of its surface immersed in the electrolyte, the latter being caused to flow at a steady rate through the system. A scraper 70 27 is arranged to collect the metallic tin 70 from the surface of the drum.

A form of construction including two cathode drums is indicated in Fig. 3, in which the anodes are constructed of easily removable elements 1, 2 and 3, each independently clamped down on to a rubber mat 4 by a series of set screws or similar clamping means in conjunction with copper connecting plates 5, 6 and 7. The two elements 1 and 3 are formed with sloping lower 80 edges so that the element 2 will contribute to hold them firmly in position.

Communicating ways 8, 9 and 10 as in Fig. 1, are provided, but the electrolyte is in this case adapted to enter simultaneously 85 through 8 and 10, and pass via annuli 11 and 12 to the outlet 9 and flow pipe 13. The two drums are rotated relatively in opposite directions as indicated by arrows. The direction of rotation may be reversed, 90 but we prefer that this shall always be such that the periphery of the drums travel in the same direction as the flow of electrolyte. Ducts 18 and 19 are provided for draining off the electrolyte when required. 95

Sloping plates 14 and 15 are provided for conveying the tin from the surface of the drums 3 and rotating wipers comprising say four rubber flaps 16 mounted to rotate on spindles 17. These wipers act to propel 100 the tin along the plates 14 and 15, and prevent it from piling up at the edge of the plates.

We prefer to construct the rotating cathode of carbon impregnated with paraffin 105 wax to enable the non-coherent metal readily to be removed and to mount it on its spindle so as to be removable readily therefrom for replacement.

Having now described our invention, what 110 we claim as new and desire to secure by Letters Patent is:—

1. An electrolytic cell comprising a casing 115 a rotatable cathode and a hollowed out anode in which the cathode may be rotated and suitable passages through the anode and casing for circulation of the electrolyte.

2. A cell such as claimed in claim 1 in which the cathode is a cylinder of carbon.

3. A cell such as claimed in claim 1 in 120 which the hollowed out anode is provided with a weir or weirs adjustable for determining the height of the electrolyte in the cell.

4. A cell such as claimed in claim 1 provided with a scraper chute to remove the deposit from the cathode.

5. An electrolytic cell comprising a cas-

ing, a cathode and an anode, the anode and casing having suitable passages therethrough for circulation of the electrolyte.

6. A cell such as claimed in claim 5 having a weir to regulate the height of the electrolyte in the cell.

7. A cell such as claimed in claim 5 in which the anode is secured to the casing by

means of a rod or rods passing through both anode and casing. <sup>10</sup>

In testimony whereof we have signed our names to this specification.

MATTHEW ATKINSON ADAM.

JOHN STEVENSON.

ALAN THOMAS MABBITT.

JOHN FIELDHOUSE.